

30 Jan  
120

# United States Patent Office

2,959,555

Patented Nov. 8, 1960

1

2,959,555

**COPPER AND IRON CONTAINING SCALE  
REMOVAL FROM FERROUS METAL**

Robert C. Martin, Tulsa, Okla., and William T. Abel, Toledo, Ohio, assignors to The Dow Chemical Company, Midland, Mich., a corporation of Delaware

No Drawing. Filed May 23, 1957, Ser. No. 660,999

6 Claims. (Cl. 252—149)

The invention relates to a method of removing from a ferrous metal surface iron oxide incrustations containing copper such as the copper-containing iron oxide incrustations oftentimes found on the internal surfaces of steam generators operated in conjunction with condensing equipment having a condensing surface of a copper alloy.

Attempts to remove copper-containing iron oxide incrustations of the type indicated above which are found quite frequently nowadays, especially in high pressure steam generators, as by chemical means, are fraught with difficulty. The use of hydrochloric acid solution is ineffective, because, although the iron oxides encountered can be removed by the acid solution, the copper component of the incrustations either is not removed or if removed by the solution is merely redeposited from it as a plating upon the ferrous metal surface. This difficulty in the use of an acid solution to remove boiler incrustations containing copper is disclosed in U.S. Patent 2,567,835 which provides a method for overcoming the difficulty. According to the patent, the incrustations can be removed by subjecting them first to the action of hydrochloric acid solution containing a corrosion inhibitor followed by a water rinse; secondly to the action of an ammoniacal solution containing a strong oxidizing agent followed by a water rinse; third to the action of dilute hydrochloric acid; and fourth to the action of a hot dilute aqueous alkaline solution. Although the foregoing method accomplishes the desired objective of removing both the iron oxide and copper components of the incrustations it has the disadvantage of requiring a multiplicity of steps which are not only laborious but also excessively time-consuming.

It is the principal object of the present invention to provide a method of removing from ferrous metal surfaces copper-containing iron oxide incrustations rapidly with a minimum of labor.

Other objects and advantages will become apparent from the following description of the invention.

According to the present invention, a copper-containing iron oxide incrustation on a ferrous metal surface, e.g. the inside of a steam generator, condenser, heat exchanger and the like, is removed by subjecting the incrustation to the action of a suitable acid solution in which is dissolved one of the following derivatives of urea: thiourea, 1,3-dimethyl thiourea, ethylene thiourea, 1,3-diethyl thiourea, and 1,3-diisopropyl thiourea. Acids capable of dissolving the iron oxides and copper-containing incrustations may be used, for example, hydrochloric acid (preferably in a concentration of 5 to 25 percent by weight), sulfuric acid (preferably in a concentration of 5 to 15 percent), and phosphoric acid (preferably in a concentration of 10 to 25 percent).

The acid solution containing the urea derivative is put into contact, in any suitable manner, with the incrustation to be removed. In treating the inside of a vessel, for example, such as a steam boiler, it may be more or less filled with the solution so as to cover the incrustations. Very large vessels may hold much more of the

2

solution than is needed to remove the incrustations. In such cases, it is more economical of solution to direct a stream of it against the incrustations instead of filling the vessel.

5 The temperature of the acid solution at which the desired copper and iron oxide removal action is obtained, without redeposition of the copper, is between about 75° F. and 160° F. Because of the temperature requirement, it may be necessary in some cases to supply heat to the solution or the equipment to be cleaned or to both the solution and the equipment to ensure having the incrustations and the solution in contact with them at a temperature at which they will be reacted upon the solution and removed.

15 Tests of the action of the solution on copper-containing iron oxide incrustations indicate that the urea derivative in the acid solution forms a precipitate or a complex with the copper which prevents it from being redeposited from the acid solution on the ferrous metal which redeposition occurs in the absence of the urea derivative.

20 The amount of the urea derivative required depends upon the quantity of copper in the incrustations to be removed and which becomes dissolved in the acid solution in the incrustation removal operation. The amount of 25 the urea derivative, we have found, should be at least about 2.0 pounds per pound of copper to be brought into solution from the incrustations by the acid. Greater amounts of the urea derivative may be used if desired, e.g. up to 20 pounds per pound of copper. The preferred 30 operating amount of the urea derivative is between about 2.2 and 6 pounds per pound of copper to be removed. It is preferable to employ at least 0.01 percent of the thiourea derivative in the solution.

35 Test data set forth in the table are illustrative of the action of various amounts of a derivative of urea (e.g. thiourea) in preventing the deposition of copper on mild steel exposed to the descaling action of hydrochloric acid containing dissolved iron oxide and cuprous chloride. In these tests, pieces of mild steel, 2.75" x 1" x 0.125", 40 were immersed for 6 hours in 150 ml. of 5 percent hydrochloric acid containing 0.4 percent of pyridine at 150° F. in which  $Fe_3O_4$ , 1.33 percent by weight, and cuprous chloride, 0.33 percent Cu by weight, were dissolved.

Table

| Test No. | Percent Thiourea | Ratio <sup>1</sup> | Observations              |                                |
|----------|------------------|--------------------|---------------------------|--------------------------------|
|          |                  |                    | Appearance of Steel Piece | Appearance of Acid Solution    |
| 50       |                  |                    |                           |                                |
| 1        | 0                | 0                  | Cu plated on steel.       | Heavy precipitate in solution. |
| 2        | 0.53             | 1.6                | Slight Cu plating.        | Do.                            |
| 3        | 0.6              | 1.8                | do                        | Light precipitate in solution. |
| 4        | 0.67             | 2.0                | Very slight Cu plating.   | Some precipitate in solution.  |
| 55       |                  |                    |                           |                                |
| 5        | 0.73             | 2.2                | No Cu plating.            | Trace precipitate in solution. |
| 6        | 0.87             | 2.6                | do                        | Do.                            |
| 7        | 0.93             | 2.8                | do                        | Do.                            |
| 8        | 1.86             | 5.6                | do                        | No precipitate in solution.    |
| 9        | 2.0              | 6.0                | do                        | Do.                            |
| 60       |                  |                    |                           |                                |
| 10       | 2.06             | 6.2                | do                        | Do.                            |
| 11       | 2.2              | 6.6                | do                        | Do.                            |

<sup>1</sup> Ratio of the amount of the thiourea to that of the copper in the acid solution.

65 From the foregoing data, it is manifest that as the concentration of the urea derivative exceeds about 0.6 percent by weight of the acid solution and the ratio of the amount of the urea derivative to that of the copper in the acid solution exceeds about 2.0 plating out of 70 copper from the acid solution onto the steel is substantially suppressed. Also it appears that the urea derivative, at the lower concentrations, forms a more or less

insoluble compound with the dissolved copper, the compound becoming a precipitate in the acid solution; and at higher concentrations the urea derivative retains the copper in solution in some form of urea-copper complex, since the copper-containing precipitate formed at lower concentrations of the urea derivative does not form at the higher concentrations of the urea derivative. In either case, that is whether the copper is converted into a precipitate in the acid solution or completely solubilized as on being complexed with the urea derivative, complete removal of the incrustations including the copper is obtained. In some cases, it is advantageous to use enough of the urea derivative to completely solubilize the copper as when the incrustations are on the inside of vessels of complex shape where the removal of a precipitate may be somewhat difficult. In most instances, it is sufficient to employ but a few pounds of the urea derivative for each pound of copper to be removed.

Other urea derivatives already mentioned may be similarly used as exemplified in the comparative tests including blanks tabulated in Table II. In these tests mild steel coupons 2.75" x 1" x 0.125" were immersed in 5 percent hydrochloric acid solutions containing 0.128 percent of cuprous chloride and 0.4 percent of pyridine for 6 hours at 150° F. The appearance of the coupons after the 6 hours immersion was observed for the effect of various thiourea derivatives added to the solution on controlling copper deposition on the coupons.

Table II

| Test No. | Thiourea Derivative <sup>1</sup>  | Appearance of Coupon       |
|----------|-----------------------------------|----------------------------|
| 12 blank | none                              | heavy copper plating.      |
| 13.      | thiourea                          | no copper plating.         |
| 14.      | 1,3-dimethyl thiourea             | negligible copper plating. |
| 15.      | ethylene thiourea                 | Do.                        |
| 16.      | 1,3-diethyl thiourea              | Do.                        |
| 17.      | 1,3-diisopropyl thiourea          | Do.                        |
| 18 blank | 1,3-dibutyl thiourea <sup>2</sup> | copper plating.            |
| 19 blank | diphenyl thiourea                 | Do.                        |
| 20 blank | dithiobiuret                      | Do.                        |

<sup>1</sup> Concentration 1.68 moles per mole of copper.

<sup>2</sup> When 1,3-dibutyl thiourea is used in combination with thiourea no copper plating occurs.

In similar tests with other concentrations of copper and other ratios of the amount of the urea derivative to the amount of copper in solution similar results were obtained as noted in the tabulation of tests in Table III carried out in similar manner to those of Table II.

Table III

| Test No. | Thiourea Derivative             | Ratio of Lbs.<br>Thiourea<br>Derivative/<br>Lb. of copper | Result             |
|----------|---------------------------------|-----------------------------------------------------------|--------------------|
| 21       | 0.34% 1,3-diethyl thiourea.     | 2.66                                                      | no copper plating. |
| 22       | 0.448% 1,3-dibutyl thiourea.    | 3.50                                                      | Do.                |
| 24       | 0.64% 1,3-diisopropyl thiourea. | 5.0                                                       | Do.                |
| 25       | 0.776% diphenyl thiourea.       | 6.06                                                      | copper plating.    |

Although the acid solution containing the urea derivative may be used without a corrosion inhibitor, the presence of a corrosion inhibitor of the organic nitrogen-base type has been found desirable especially when operating at temperatures much above 80° F.

Common organic nitrogen bases which may be used as inhibitors are the well known coal tar bases produced in the distillation of coal tar. If desired the bases themselves may be separated from the crude coal tar base mixture and used as individual substances. These compounds are the aromatic and heterocyclic nitrogen bases soluble in the acid solution. The concentration or amount of the organic nitrogen-base inhibitor to em-

ploy depends upon its effectiveness and the extent to which it is desired to suppress the corrosiveness of the acid and the temperature at which the acid solution is to be used. Generally the amount effective to inhibit or reduce the corrosiveness of the acid is in the range of 0.1 to 1 percent of the weight of the acid solution.

The following are examples of corrosion inhibitors from coal tar: pyridine, alpha-picoline, beta-picoline, gamma-picoline, 2-n-amylopyridine, 4-n-amylopyridine, 2-hexyl-pyridine, 2,4-lutidine, 2,6-lutidine, 2,4,6-collidine, quinoline, lepidine, quinaldine. Other compatible organic nitrogen-base inhibitors are rosin amines and hydrogenated rosin amines (see U.S. Patent 2,510,063 and 2,510,284).

The following example is illustrative of the practice of the invention as applied to cleaning a steam generator (high pressure steam boiler) having an internal volume of about 20,000 gallons. Prior to cleaning, examination of the interior of the generator revealed extensive incrustations of ferrosoferric oxide estimated to amount to about 2000 pounds. Occluded in the incrustations was an amount of copper and copper oxide estimated to be the equivalent of about 150 pounds of metallic copper. To remove these copper-containing iron oxide incrustations, the generator was filled with a water solution of hydrochloric acid containing 5 percent of HCl, 2400 pounds of thiourea in solution, and 0.4 percent of pyridine as a corrosion inhibitor. After filling the generator with the foregoing solution, it was heated so as to bring the temperature of the generator and the acid solution in it to about 150° F. and this temperature was maintained for about 6 hours. During this time the iron oxide and copper incrustations were dissolved by and retained in the acid solution without any redeposition of the copper on the internal surfaces of the generator.

35 The resulting spent acid solution was drained out of the generator which was then flushed with water. Examination revealed that the incrustations were removed leaving the interior surfaces clean and copper free.

The so-cleaned generator was then refilled with a dilute 40 soda ash solution (about 3 percent Na<sub>2</sub>CO<sub>3</sub>) which was then boiled for two hours in the generator to remove any trace of the acid solution. The generator was then drained and flushed with water.

As is evident from the examples given herein, the 45 solution of metallic copper in the acid solution occurs in the presence of ferric iron derived from the iron oxide in the incrustations. This reaction may be expressed by the equation:



50 in which the metallic copper is converted into a cuprous compound. In the presence of the urea derivative used in accordance with the invention the copper so dissolved is precluded from redepositing upon a ferrous metal surface. While we have found that most copper containing incrustations to be removed by the acid solution contain an adequate amount of ferric iron to oxidize the copper a deficiency, if any, of ferric iron in the incrustation can be made up by adding a suitable oxidizing agent to the acid solution.

55 For example, there may be used iron oxide (Fe<sub>2</sub>O<sub>3</sub> or Fe<sub>3</sub>O<sub>4</sub>) or ferric chloride as an oxidizing agent in amount sufficient to meet the stoichiometric requirements of the foregoing equation.

60 Among the advantages of the method are that a single 65 solution suffices to remove the incrustations. Since only one cleaning step is involved, the down time of the equipment to be cleaned is reduced to a minimum.

This application is a continuation-in-part of our 70 pending application Serial No. 612,894, filed September 28, 1956, now abandoned.

We claim:

1. The method of removing copper and iron oxide containing incrustation from a ferrous metal surface without 75 redeposition of copper thereon which consists in bringing into contact with such surface an aqueous solution of a

urea derivative selected from the group consisting of thiourea, 1,3-dimethyl thiourea, ethylene thiourea, 1,3-diethyl thiourea, and 1,3-diisopropyl thiourea, said solution containing an acid capable of dissolving the iron oxides and copper, the amount of said urea derivative being from 2 to 20 pounds per pound of copper in the incrustation, said aqueous solution being maintained in contact with the incrustation for a time sufficient to substantially solubilize the said incrustation.

2. The method according to claim 1 in which the aqueous solution also contains an amount of an organic nitrogen-base other than thiourea and the substituted thiourea compounds defined in claim 1 capable of inhibiting the corrosive action of the acid on ferrous metal.

3. The method of removing a copper and iron oxide containing incrustation from a ferrous metal surface without redeposition of copper thereon which consists in bringing into contact with such surfaces an aqueous solution consisting of water in which is dissolved from 5 to 25 percent by weight of hydrochloric acid, thiourea, and from 0.1 to 1 percent of an organic nitrogen base other than thiourea capable of inhibiting the corrosive action of the acid on ferrous metal, the amount of the thiourea being in excess of 0.01 percent by weight of the solution and between 2 and 20 times the weight of the copper to be removed, the volume of the aqueous solution being sufficient to remove the incrustations.

4. A composition for removing copper containing iron oxide incrustations from a ferrous metal surface consisting of a solution in water of from 2 to 25 percent by weight of hydrochloric acid, a urea derivative selected from the group consisting of thiourea, 1,3-dimethyl

thiourea, ethylene thiourea, 1,3-diethyl thiourea, 1,3-diisopropyl thiourea in the amount of at least 0.67 percent by weight, and from 0.1 to 1 percent of an organic nitrogen base soluble in the solution selected from the group consisting of the aromatic and heterocyclic nitrogen bases capable of inhibiting the corrosive action of the acid on ferrous metal.

5. The method according to claim 3 in which there is included in the aqueous solution an oxidizing agent capable of oxidizing the copper in the incrustation to the cuprous state.

6. The method according to claim 5 in which the oxidizing agent is ferric chloride.

15 References Cited in the file of this patent

UNITED STATES PATENTS

|                |                                     |                |
|----------------|-------------------------------------|----------------|
| — 1,961,096    | Cunningham <del>2,52-149</del>      | May 29, 1934   |
| — 1,996,730    | Thomas et al. <del>2,52-147</del>   | Apr. 2, 1935   |
| — 2,049,517    | Saukaitis <del>2,52-149</del>       | Aug. 4, 1936   |
| 20 2,071,966   | Bolton <del>2,52-149</del>          | Feb. 23, 1937  |
| 2,215,077      | Beekhuis et al. <del>2,52-142</del> | Sept. 17, 1940 |
| — 2,220,451    | Hunt <del>2,52-142</del>            | Nov. 5, 1940   |
| — 2,318,559    | Percival <del>2,52-142</del>        | May 4, 1943    |
| 25 2,474,526   | Healy et al. <del>2,52-142</del>    | June 28, 1949  |
| — 2,485,529    | Cardwell et al. <del>2,52-142</del> | Oct. 18, 1949  |
| — 2,617,771    | Rucker <del>2,52-142</del>          | Nov. 11, 1952  |
| — 2,618,603    | Schaeffer <del>2,52-142</del>       | Nov. 18, 1952  |
| — 2,628,199    | Lowenheim <del>2,52-142</del>       | Feb. 10, 1953  |
| 30 — 2,769,690 | Mahan et al. <del>2,52-142</del>    | Nov. 6, 1956   |

504,269

FOREIGN PATENTS

Belgium ~~2,52-148~~ July 14, 1951